

## UNITED STATES PATENT OFFICE

2,157,390

## METHOD FOR MAKING CAST IRON

William J. Priestley, New Rochelle, N. Y., assignor to Electro Metallurgical Company, a corporation of West Virginia

No Drawing. Application January 25, 1937,  
Serial No. 122,235

9 Claims. (Cl. 75—58)

The invention relates to cast iron and provides a novel method and means for improving cast irons of all varieties. The invention will be described in connection with gray cast iron made in the cupola with little or no steel in the charge; but the invention is equally suitable for use to improve all varieties of cast iron, including white and mottled iron and irons of mixed or graded structures, when made in any type of furnace from any kind of charge.

Sources of weakness in gray cast iron are the formation of large graphite flakes and large grains in heavy sections, too deep a chill in light sections, and too large an amount of "eutectic" graphite in sections behind a chill. An ideal gray cast iron would have a uniform fine-grained structure, uniform chill characteristics, and fine flake graphite uniformly distributed.

It is well known that the chilling characteristics of a cast iron may sometimes be reduced by a relatively small addition of graphite in the forehearth or ladle. This effect is accompanied, however, by a softening of the metal and, in some cases, by a decrease in its tensile and transverse strengths. These effects are illustrated by the data in Table A.

Table A

| No. | Ladle addition | Analysis of cast iron |            |            | Tensile strength, lb/sq. in. | Transverse strength, lb/sq. in. | Deflection, inches | Brinell hardness number |
|-----|----------------|-----------------------|------------|------------|------------------------------|---------------------------------|--------------------|-------------------------|
|     |                | T. C. percent         | Percent Si | Percent Mn |                              |                                 |                    |                         |
| 1   | None           | 2.95                  | 2.98       | 0.6        | 31,160                       | 3,620                           | 0.18               | 170                     |
| 2   | Graphite*      | 3.05                  | 2.85       | 0.6        | 30,425                       | 3,100                           | 0.15               | 166                     |

\* 4 ounces of graphite per 100 pounds of metal.

It is also known that the chilling characteristics can be reduced by adding silicon or zirconium, in small amounts, in cupola, forehearth, or ladle. In order to secure markedly improved results by this means, however, it is necessary to use so much of the silicon addition that the composition is changed substantially, and the base mixture must be altered to compensate for this change so that the correct final composition will be obtained. Sometimes, the chill in light sections of a casting cannot be suppressed by this expedient without producing undesirably coarse graphite in the heavier section.

On occasion, both ferrosilicon (containing 50% silicon) and graphite have been added to cast iron, almost simultaneously but not in admixture. As would be expected, the effects of the two ma-

terials are substantially additive when they are added in this fashion.

I have discovered that if graphite, or other form of carbon, is intimately mixed with silicon or zirconium, or both, and this intimate mixture is added in relatively small amount to a molten cast iron, the iron is improved to an extent, and in a manner, quite different from what could be predicted from the previous knowledge of the individual effects of the constituents of the mixture.

Specifically, such a mixture refines the grain and the graphite flakes in heavy sections, reduces or eliminates chill, suppresses or inhibits the formation of eutectic graphite, inhibits the formation of an open grain structure inside heavy sections, and raises the tensile and transverse strength without greatly altering the ductility or hardness of the main body of the casting, the effects obtained depending, of course, on the composition of the melt and the casting conditions.

Although graphite is preferred as the carbonaceous ingredient of the mixture, because of its ready solubility in molten iron, other forms of carbon, such as charcoal, coal coke, petroleum

coke, or carbon black, may be used. The silicon or zirconium may be used in any of the commercial forms of these elements, such as silicon metal, ferrosilicon, or silicon-zirconium alloy. When ferrosilicon is used, it is particularly advantageous to use a ferrosilicon containing at least 65% silicon. Ferrosilicon having a lower proportion of silicon appears to cool the iron at least locally, while those having at least 65% silicon generate enough heat by exothermic reaction to counteract any cooling effect.

A mixture of approximately equal parts by weight of graphite and 85% grade ferrosilicon will be found to be of most general suitability, although mixtures containing other proportions may be used. If a relatively large amount of the mixture is employed, the proportions may range from 5% carbon and 95% ferrosilicon or its

equivalent, to 95% carbon and 5% ferrosilicon or its equivalent; but if only a small amount of mixture is used, the proportions should be between 25% and 75% carbon, remainder ferrosilicon or its equivalent.

The ingredients of the mixture should be finely subdivided and intimately mixed. Particle sizes from that just passing a three mesh screen to fine powder have been used successfully, and somewhat larger particles are useful. The mixture may be used as loose grains or powder.

The amount of mixture to be added will vary, of course, with the type of cast iron and the intensity of the effect desired; but in no case need it be sufficient to alter substantially the chemical composition of the cast iron. Additions of 4 to 8 ounces of the mixture for each 100 pounds of cast iron have given excellent results; but smaller or larger amounts, between the approximate limits of 1 to 16 ounces per 100 pounds of cast iron, are useful, the upper limit being set chiefly by considerations of economy and change of composition.

The benefits conferred by the invention are illustrated by the data appearing in Table B:

Table B

| No. | Ladle addition | Analysis of cast iron |               |            | Tensile strength, lb/sq. in. | Transverse strength, lb/sq. in. | Deflection, inches | Brinell hardness number |
|-----|----------------|-----------------------|---------------|------------|------------------------------|---------------------------------|--------------------|-------------------------|
|     |                | Percent Si            | T. C. percent | Percent Mn |                              |                                 |                    |                         |
| 3   | None           | 1.58                  | 2.95          | 0.6        | 32,785                       | 3,390                           | 0.09               | 220                     |
| 4   | *              | 1.56                  | 3.05          | 0.6        | 38,080                       | 3,730                           | 0.10               | 239                     |
| 5   | **             | 1.62                  | 2.90          | 0.6        | 40,400                       | 3,750                           | 0.11               | 228                     |
| 35  | None           | 1.84                  | 3.16          | 0.7        | 37,180                       | 2,340                           | 0.22               | -----                   |
| 6   | **             | 1.95                  | 3.20          | 0.7        | 40,160                       | 2,800                           | 0.30               | -----                   |
| 7   | None           | 1.95                  | 3.18          | 0.8        | -----                        | 2,220                           | 0.19               | -----                   |
| 8   | *              | 1.98                  | 3.24          | 0.8        | -----                        | 2,760                           | 0.28               | -----                   |
| 9   | None           | 2.98                  | 2.95          | 0.6        | 31,160                       | 3,620                           | 0.18               | 170                     |
| 10  | *              | 2.98                  | 2.95          | 0.6        | 40,500                       | 3,740                           | 0.13               | 223                     |

\* 4 ounces of addition mixture per 100 pounds of cast iron.  
\*\* 8 ounces of addition mixture per 100 pounds of cast iron.

Addition mixture consisted of equal parts by weight of graphite and ferrosilicon containing 85% Si.

In Tables A and B, the symbol "T. C." means total carbon; and tensile strength and transverse tests were made in accordance with the standard A. S. T. M. specifications. The transverse tests on samples 6, 7, 8, and 9 were made on supports 18 inches apart; on the remaining samples, on supports 12 inches apart.

The presence of large amounts of strong carbide-forming elements, in the cast iron, such as more than 10% of chromium, masks or destroys the beneficial effects of the invention by preventing graphitization of the combined carbon.

The chill ordinarily produced in low-silicon irons by the presence of a high sulfur content is reduced or eliminated by the use of the addition mixture of the invention. For instance, a melt of white-iron composition containing 0.75% silicon, 0.28% manganese, 0.31% sulfur, 0.143% phosphorus, 2.86% carbon, remainder iron, was treated by the addition of a small amount of the addition mixture referred to in Table B, and the melt cast. The casting was found to be a mottled iron instead of a white iron.

Modifications of the invention as described herein will readily occur to those skilled in the art. Accordingly, the invention is not limited to the specific examples mentioned above by way of example.

I claim:

1. Method of increasing the strength of cast iron which comprises adding to a molten cast iron an unbonded intimate mixture containing 25% to 75% carbon and at least one element

selected from the group consisting of silicon and zirconium, the amount of said mixture added being between one and sixteen ounces for each 100 pounds of molten cast iron; and casting the melt.

2. Method of making cast iron which comprises adding to a molten cast iron an effective amount of an unbonded intimate mixture containing 25% to 75% graphite and the remainder principally ferrosilicon containing at least 65% silicon, the amount of said mixture added being insufficient to change substantially the chemical composition of said molten iron, and casting the melt.

3. Method of making cast iron which comprises adding to a molten cast iron an effective amount of an unbonded intimate mixture consisting essentially of graphite and ferrosilicon in substantially equal amounts by weight, the ferrosilicon containing at least 85% silicon, the amount of said mixture added being insufficient to change substantially the chemical composition of said molten iron, and casting the melt.

4. The method of reducing the chill of a high-sulfur, low-silicon cast iron containing not less

25

30

35

40

45

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

1005

1010

1015

1020

1025

1030

1035

1040

1045

1050

1055

1060

1065

1070

1075

1080

1085

1090

1095

1100

1105

1110

1115

1120

1125

1130

1135

1140

1145

1150

1155

1160

1165

1170

1175

1180

1185

1190

1195

1200

1205

1210

1215

1220

1225

1230

1235

1240

1245

1250

1255

1260

1265

1270

1275

1280

1285

1290

1295

1300

1305

1310

1315

1320

1325

1330

1335

1340

1345

1350

1355

1360

1365

1370

1375

1380

1385

1390

1395

1400

1405

1410

1415

1420

1425

1430

1435

1440

1445

1450

1455

1460

1465

1470

1475

1480

1485

1490

1495

1500

1505

1510

1515

1520

1525

1530

1535

1540

1545

1550

1555

1560

1565

1570

1575

1580

1585

1590

1595

1600

1605

1610

1615

1620

1625

1630

1635

1640

1645

1650

1655

1660

1665

1670

1675

1680

1685

1690

1695

1700

1705

1710

1715

1720

1725

1730

1735

1740

1745

1750

1755

1760

1765

1770

1775

1780

1785

1790

1795

1800

1805

1810

1815

1820

1825

1830

1835

1840

1845

1850

1855

1860

1865

1870

1875

1880

1885

1890

1895

1900

1905

1910

1915

1920

1925

1930

1935

1940

1945

1950

1955

1960

1965

1970

1975

1980

1985

1990

1995

2000

2005

2010

2015

2020

2025

2030

2035

2040

2045

2050

2055

2060

2065

2070

2075

2080

2085

2090

2095

2100

2105

2110

2115

2120

2125

2130

2135

2140

2145

2150

2155

2160

2165

2170

2175

2180

2185

2190

2195

2200

2205

2210

2215

2220

2225

2230

2235

2240

2245

2250

2255

2260

2265

2270

2275

2280

2285

2290

2295

2300

2305

2310

2315

2320

2325

2330

2335

2340

2345

2350

2355

2360

2365

2370

2375

2380

2385

2390

2395

2400

2405

2410

2415

2420

2425

2430

2435

2440

2445

2450

2455

2460

2465

2470

2475

2480

2485

2490

2495

2500

2505

2510

2515

2520

2525

2530

2535

2540

2545

2550

2555

2560

2565

2570

2575

2580

2585

2590

2595

2600

2605

2610

2615

2620

2625

2630

2635

2640

2645

2650

2655

2660

2665

2670

2675

2680

2685

2690

2695

2700

2705

2710

2715

2720

2725

2730

2735

2740

2745

2750

2755

2760

2765

2770

2775

2780

2785

2790

2795

2800

2805

2810

2815

2820

2825

2830

2835

2840

2845

2850

2855

2860

2865

2870

2875

2880

2885

2890

2895

2900

2905

2910

2915

2920

2925

2930

2935

2940

2945

2950

2955

2960

2965

2970

2975

2980

2985

2990

2995

3000

3005

3010

3015

3020

3025

3030

3035

3040

3045

3050

3055

3060

3065

3070

3075

3080

3085

3090

3095

3100

3105

3110

3115

3120

3125

3130

3135

3140

3145

3150

3155

3160

3165

3170

3175

3180

3185

3190

3195

3200

3205

3210

3215

3220

3225

3230

3235

3240

3245

3250

3255

3260

3265

3270

3275

3280

3285

3290

3295

3300

3305

3310

3315

3320

3325

3330

3335

3340

3345

3350

3355

3360

3365

3370

3375

3380

3385

3390

3395

3400

3405

3410

3415

3420

3425

3430

3435

3440

3445

3450

3455

3460

3465

3470

3475

3480

3485

3490

3495

3500

3505

3510

3515

3520

3525

3530

3535

3540

3545

3550

3555

3560

3565

3570

3575

3580

3585

3590

3595

3600

3605

3610

3615

3620

3625

3630

3635

3640

3645

3650

3655

3660

3665

3670

3675

3680

3685

3690

3695

3700

3705

3710

3715

3720

3725

3730

3735

3740

3745

3750

3755

3760

3765

3770

3775

3780

3785

3790

3795

3800

3805

3810

3815

3820

3825

3830

3835

3840

3845

3850

3855

3860

3865

3870

3875

3880

3885

3890

3895

3900

3905

3910

3915

3920

3925

3930

3935

3940

3945

3950

3955

3960

3965

3970

3975

3980

3985

3990

3995

4000

4005

4010

4015

4020

4025

4030

4035

4040

4045

4050

4055

4060

4065

4070

4075

4080

4085

4090

4095

4100

4105

4110

4115

4120

4125

4130

4135

4140

4145

4150

4155

4160

4165

4170

4175

4180

4185

4190

4195

4200

4205

4210

4215

4220

4225

4230

4235

4240

4245

4250

4255

4260

4265

4270

4275

4280

4285

4290

4295

4300

4305

4310

4315

4320

4325

4330

4335

4340

4345

4350

4355

4360

4365

4370

4375

4380

4385

4390

4395

4400

4405

4410

4415

4420

4425

4430

4435

4440

4445

4450

4455

4460

4465

4470

4475

4480

4485

4490

4495

4500

4505

4510

4515

4520

4525

4530

4535

4540

4545

4550

4555

4560

4565

4570

4575

4580

4585

4590

4595

4600

4605

4610

4615

4620

4625

4630

4635

4640

4645

4650

4655

4660

4665

4670

4675

4680

4685

4690

4695

4700

4705

4710

4715

4720

4725

4730

4735

4740

4745

4750

4755

4760

4765

4770

4775

4780

4785

4790

4795

4800

4805

4810

4815

4820

4825

4830

4835

4840

4845

4850

4855

4860

4865

4870

4875

4880

4885

4890

4895</

least 65% silicon; the proportions of graphite and ferrosilicon in said mixture being approximately equal by weight, and the amount of said mixture added being insufficient to change substantially the chemical composition of said molten iron; and casting the melt.

8. An agent for treating molten cast-iron in a forehearth or ladle, consisting of an unbonded intimate admixture of powdered materials and composed wholly of carbon and material selected

from the group: silicon, ferrosilicon, zirconium, and silicon-zirconium; the carbon being between 25% and 75% of the agent.

9. An agent for treating molten cast-iron in a forehearth or ladle, consisting entirely of an unbonded intimate admixture of powdered graphite and powdered ferrosilicon in approximately equal parts by weight.

WILLIAM J. PRIESTLEY. 10